

## UNITED STATES PATENT OFFICE

2,524,741

MAGENTA PHENAZONIUM DYESTUFF  
IMAGES FROM 6-SUBSTITUTED-8-HYDROXYQUINOLINE COUPLERS

Vsevolod Tulagin, Phillipsburg, N. J., and Robert F. Coles, Easton, Pa., assignors to General Aniline &amp; Film Corporation, New York, N. Y., a corporation of Delaware

No Drawing. Application December 23, 1947,  
Serial No. 793,533

5 Claims. (Cl. 95—6)

1

The present invention relates to the production of phenazonium dyestuff images by color development of exposed silver halide emulsions by means of derivatives of ortho-phenylene diamine, and more particularly to the employment in such process of color formers which directly yield the phenazonium dyestuff images by such color development.

Schmidt and Tulagin copending application Ser. No. 640,382, filed January 10, 1946, now Patent No. 2,486,440, describes the production of phenazonium dyestuff images by color developing an exposed silver halide emulsion with a color developer comprising a developer of the ortho-phenylene diamine type in the presence of 8-hydroxy-quinoline as the color former.

The phenazonium dye images produced in this way are extremely desirable from the standpoint of transmission spectra and stability. However, the phenazonium dyes of such images are only formed by a special after-treatment with acids or alkalies of the green dye image, presumably of a quinoneimine, resulting from the color forming development step. The value of the phenazonium dye as a photographic image is therefore somewhat offset by the fact that additional time and chemicals are necessary in order to obtain the image thereof.

It has now been found that such dye images can be directly produced by the color forming development step, i. e., without an additional after-treatment if there be employed as the color former 8-hydroxy-quinolines (including 8-hydroxy cinchoninic acids) containing in the —6 position of the quinoline ring a substituent which is eliminated during the color forming development as a negative ion. The utilization of such color formers in the production of phenazonium dyestuff images and silver halide emulsions containing the same accordingly constitute the purposes and objects of the present invention.

The color formers contemplated herein are characterized by the following general formula:



wherein R is halogen, i. e., bromine, chlorine, iodine, or the like, nitro, sulfo, or an arsonic acid radical, R<sub>1</sub> is hydrogen, alkyl or a mononuclear carbocyclic aromatic radical such as phenyl, 55

2

nitrophenyl, aminophenyl, stearoylaminophenyl, octadecanesulfonamidophenyl, chlorophenyl, tolyl, anisyl and the like, R<sub>2</sub> is hydrogen, —COOH or —CONHR<sub>3</sub> and R<sub>3</sub> is a sulfonated aliphatic radical containing at least 10 carbon atoms or a sulfonated aromatic radical substituted by an aliphatic radical containing at least 10 carbon atoms.

Examples of compounds embraced by the above formula are the following:

1.



15

2.



20

3.



25

4.



35

40

5.



45

6.

50



3



15.

5



2-(3-octadecanesulfonamidophenyl)-6-bromo-8-hydroxycinchoninic acid

10.

15.



2-(4-chlorophenyl)-6-bromo-8-hydroxycinchoninic acid

20.

25.



2-(4-tolyl)-6-bromo-8-hydroxycinchoninic acid

18.

30.



2-(4-methoxyphenyl)-6-bromo-8-hydroxycinchoninic acid

35. It will be apparent that in the compounds listed above, those containing the long aliphatic chain will be non-migratory when located in photographic emulsions. Consequently when the employment of these compounds is desired, they are most advantageously dispersed in emulsions. The other compounds, however, may be employed either in the developer or in the emulsion although it is preferred that they be added to the developer.

45. The color developers which are utilized are, as stated, of the ortho-phenylene diamine type, a large number of examples of which are referred to in the aforesaid Schmidt and Tulagin application. Suitable developers of this class are, for 50. example:

4,6-dianilino-metanilic acid

4,6-bis-(p-methoxy-phenylamino)-metanilic acid

4-(o-methoxy - phenylamino) - 6 - (p - methoxy-

55. phenylamino)-metanilic acid

4,6-bis-(o-methoxy phenylamino)-metanilic acid

4-(p-sulfo-phenylamino) -6-dimethylamino-met-

anilic acid

and the like.

60. Many of the color formers previously referred to are known compounds. Those which are not described in the literature, such as compounds 9 to 18, are prepared by methods conventional in the art. For instance, compound No. 9 may be 65 obtained by treating equimolecular quantities of 2-phenyl-6-bromo-8-hydroxycinchoninic acid and 6-amino-2-stearoylaminotoluene-4-sulfonic acid in pyridine solution with an excess of phosphorus trichloride. Compounds 10 and 11 can be prepared by similar procedures using the appropriate intermediates.

Compound 12 can be prepared by heating a mixture of 2-amino-5-bromophenol, m-nitrobenzaldehyde and pyruvic acid in ethyl alcohol.

75. Compound 13 can be prepared by hydrogenating

compound 12 dissolved in aqueous sodium hydroxide using a platinum oxide catalyst. Compounds 14 and 15 can be prepared by reacting compound 13 in pyridine solution with octadecanoyl chloride and octadecanesulfonyl chloride respectively. Compounds 16, 17 and 18 can be prepared by employing the procedure described for compound 12 using p-chlorobenzaldehyde, p-methylbenzaldehyde and p-methoxybenzaldehyde respectively in place of m-nitrobenzaldehyde.

The invention is illustrated by the following examples, but it is to be understood that these examples are illustrative and not limitative of the invention.

*Example 1*

A photographic silver bromide emulsion is exposed and then color developed for 5 to 10 minutes in a solution of the following color developer:

|                              |       |      |
|------------------------------|-------|------|
| Sodium carbonate monohydrate | grams | 60   |
| Potassium bromide            | do    | 2    |
| Sodium sulfite               | do    | 40   |
| Pyridine                     | cc    | 12   |
| 4,6-dianilino-metanilic acid | grams | 4    |
| 6-bromo-8-hydroxyquinoline   | do    | 2    |
| Water                        | cc    | 1000 |

A magenta phenazonium dyestuff image is directly produced by this development. By further processing the film in the usual manner, images of an excellent transmission spectra and stability are obtained.

*Example 2*

.5 gram of compound No. 9 is dissolved in 1.4 ml. of 0.05 N-lithium hydroxide, the solution diluted to 17 ml. with water and then neutralized with dilute acetic acid. The resulting solution is added to 35 grams of a photographic silver bromide emulsion and the emulsion coated on a film base.

The emulsion is then exposed and color developed with the developer of Example 1, excepting that the 6-bromo-8-hydroxyquinoline is omitted therefrom. A brilliant magenta phenazonium dyestuff image of excellent stability is directly produced in the development step.

Various modifications of the invention will occur to workers in this art, and we therefore do not intend to be limited in the patent granted except as necessitated by the prior art and the appended claims.

We claim:

1. The process of producing magenta phenazonium dyestuff images by color forming development which comprises exposing a silver halide emulsion and developing the same with a 2,4-diaminoaniline developer in the presence of a color former having the following formula:



wherein R is a member of the class consisting of halogen, nitro, sulfo and arsonic acid radicals, R<sub>1</sub> is a member of the class consisting of hydrogen, alkyl and a mononuclear carbocyclic aromatic radical, R<sub>2</sub> is a member of the class consisting of H, —COOH and —CONH—R<sub>3</sub> and R<sub>3</sub> is a member selected from the class consisting of sulfonated aliphatic radicals containing at least 10 carbon atoms, and sulfonated aromatic radicals substituted by an aliphatic radical containing at least 10 carbon atoms.

2. The process as defined in claim 1 wherein the color former is 6-sulfo-8-hydroxy quinoline.

3. The process as defined in claim 1 wherein the color former is 6-bromo-8-hydroxy-quinoline.

4. A photographic silver halide emulsion containing as a color former capable of directly yielding magenta phenazonium dyestuff images when color developed with a 2,4-diamino aniline developer, a compound of the following formula:



wherein R is a member of the class consisting of halogen, nitro, sulfo and arsonic acid radicals, R<sub>1</sub> is a member of the class consisting of hydrogen, alkyl and a mononuclear carbocyclic aromatic radical, R<sub>2</sub> is a member of the class consisting of H, —COOH and —CONH—R<sub>3</sub> and R<sub>3</sub> is a member selected from the class consisting of sulfonated aliphatic radicals containing at least 10 carbon atoms, and sulfonated aromatic radicals substituted by an aliphatic radical containing at least 10 carbon atoms.

5. A photographic silver halide emulsion containing as a color former a compound of the following formula:



VSEVOLOD TULAGIN.  
ROBERT F. COLES.

**REFERENCES CITED**

The following references are of record in the file of this patent:

**FOREIGN PATENTS**

| Number  | Country       | Date          |
|---------|---------------|---------------|
| 836,144 | France        | Oct. 10, 1937 |
| 478,986 | Great Britain | Jan. 24, 1938 |